

April 5, 1927.

1,623,271

N. C. RENDLEMAN

MANUFACTURE OF FLANGED BEAMS

Filed March 15, 1923

4 Sheets-Sheet 1



April 5, 1927.

1,623,271

N. C. RENDLEMAN

MANUFACTURE OF FLANGED BEAMS

Filed March 15, 1923

4 Sheets-Sheet 2



his Attorneys

April 5, 1927.

1,623,271

N. C. RENDLEMAN

MANUFACTURE OF FLANGED BEAMS

Filed March 15, 1923

4 Sheets-Sheet 3



Inventor

Norman C. Rendleman

By Emery, Booth, Farney & Warner

his Attorneys

April 5, 1927.

1,623,271

N. C. RENDLEMAN

MANUFACTURE OF FLANGED BEAMS

Filed March 15, 1923

4 Sheets-Sheet 4

FIG. 5.



FIG. 6.



FIG. 7.



Inventor

Norman C. Rendleman

By Emery, Booth, Janney & Narney

his Attorneys

Patented Apr. 5, 1927.

## UNITED STATES PATENT OFFICE.

NORMAN C. RENDLEMAN, OF DORMONT, PENNSYLVANIA, ASSIGNOR TO JONES & LAUGHLIN STEEL CORPORATION, OF PITTSBURGH, PENNSYLVANIA, A CORPORATION OF PENNSYLVANIA.

## MANUFACTURE OF FLANGED BEAMS.

Application filed March 15, 1923. Serial No. 625,342.

This invention aims to improve processes of metal rolling, and is particularly applicable to rolling flanged structural members and beams having thin webs, such as I-beams and channels, of light weight and greater depth in proportion to weight than it has heretofore been considered practicable to produce or than could be readily produced by rolling processes heretofore commonly used.

10 A further aim of the invention is to improve metal rolling processes whereby the necessary changes in cross-sectional shape from the billet to the finished shape may be secured with a minimum reduction in cross-sectional area, thus enabling thin sections to be completed at one heat.

Further aims and advantages of the invention appear hereinafter in connection with the illustrative mode of practicing the invention shown in the accompanying drawings, wherein—

Fig. 1 is a vertical longitudinal section through the bight of the lower pair of mating rolls of the first stand of a suitable three-high rolling mill, the view being broken into two parts in order to get it on the sheet;

Fig. 2 is a similar view of two of the mating rolls of a second stand of three-high rolls suitable for completing the beam blank ready for finishing the beam;

Fig. 3 is an end view showing the outline or shape of the cross-section of the finished beam chosen for illustrating the process;

Fig. 4 is a diagram showing full size the comparative shapes of the illustrative billet and blank at successive stages of the process;

Figs. 5 and 6 are comparative views drawn to the same scale showing the lightest weight standard I-beams heretofore rolled by existing processes and the billets or blanks from which they are produced; and

Fig. 7 is a similar view drawn to the same scale of a light weight I-beam of the same depth as those shown in Figs. 5 and 6 and the billet from which it may be produced by my process.

In the rolling of very thin sections time is an important factor as the rolling must be completed before the temperature of the metal becomes too low. My invention enables light, thin sections to be produced with fewer rolling passes than heretofore and

hence shortens the time required to the limit within which the rolling may be completed at one heat. In the rolling of beams as heretofore practiced it was impracticable to roll the very light sections to which my invention is applicable within this time limit, even by the use of special facilities and the highest rolling speeds available.

Special rolling mills are not required for practicing my invention, as suitable types of rolling mills in common use may be utilized for performing the operations comprised therein, that selected for illustration being a horizontal mill having two stands of three rolls each, commonly termed a "three-high" mill.

Referring to Figs. 1 and 2, the successive passes are respectively designated by the numerals 1 to 8, inclusive, appearing either below or above the pass, depending upon whether the beam is passed below or above the middle roll in each instance in the case selected for illustration. Also in order that the invention may be more readily understood, the outline of the cross-section of the billet or blank as it enters each pass is shown in dotted lines superposed upon the drawing of the pass in the relative position in which it enters the pass, passes 2, 4, 6 and 8 being shown inverted from their true positions.

For purposes of description the invention is illustrated in a suitable mode for the production of a ten inch I-beam 10 (see Fig. 3) having a weight of about eight pounds per linear foot and of such cross-sectional shape that the thickness of the web 11 is about  $1\frac{1}{2}\%$  of the depth, and the width of the flange 12 is about 30% of the depth.

Such a beam may advantageously be rolled from an approximately square billet whose longest side is preferably about one-half the depth of the beam (see Figs. 4 and 7). In the example selected for illustration the billet 13 is five inches square and weighs a little over eighty pounds per foot, necessitating a reduction in cross-section and consequent elongation of about ten to one. This billet is much smaller in height and width than the blooms or billets required for producing flanged beams of the same depth by any rolling methods now in use (see Figs. 5

and 6) and hence can be rolled to finished dimensions in less time than has heretofore been possible with larger billets, and while the metal is at rolling heat.

- 5 Another advantage of my process is that the smaller billet required has sufficient length to be readily handled in the heating furnaces and on the rolling mill tables; whereas the considerably larger billets or 10 blooms 21, 22 (see Fig. 5) required for producing the I-beam 23 by the "groove" process of rolling, and the equally large beam blank 24 (see Fig. 6) required for producing the I-beam 25 by rolling in a universal 15 mill, which were the only commercially practicable means heretofore available for rolling flanged beams, are either too short to be readily handled in the furnaces and on the tables in the first passes or else they produce 20 too long a finished product to be completed within the time available while the metal is at a rolling heat.

In the first pass (see upper half of Fig. 1) the roll grooves 1, 1' of the middle and 25 lower rolls are similar and are provided with central wedge shaped working collars to channel the billet 13 (shown in dotted lines in Fig. 1) on both sides along its mid-line and separate the edges so as to spread 30 the blank 30% to 50% in width, and thin its thickness at the middle 60% to 80% or more, preferably with a minimum reduction in cross-sectional area. The resulting hour 35 glass shape blank 14 (see Fig. 4) is rolled through a second pass having similarly shaped roll grooves 2, 2' calculated to thin the middle portion 30% to 60% to form a web and to spread the flanged edges to 40 expand the blank 10% to 25% more in width with a minimum reduction in cross-sectional area. This rapid deformation is made possible by permitting a considerable portion of the displaced metal to flow laterally into the flanges, as shown in Fig. 1.

45 The resulting dumb-bell shape blank 15 (see Fig. 4 and lower half of Fig. 1) may if preferred be successively rolled through one or more passes having similar but wider 50 grooves, until its width is over 90% of the depth of the finished beam and its thickness at the edges of the flanges and through the web is such that the areas of these portions exceed those of the flanges and web of the finished beam in similar proportions. In 55 the illustrative case in the first pass the billet is spread from a 5" by 5" square to a width of 7" (about 40% increase in width) and is reduced in thickness at the middle to 1 1/8" (a reduction of about 77 1/2%), and in 60 the second pass the width is increased to 8 3/8" (about 19.6%) and the thickness is reduced to 5/8" (about 44.4%), the total spreading in the two passes being about 67 1/2% and the reduction in thickness of the 65 web being about 87 1/2% of the original di-

mensions of the billet. By rolling the billet in this manner it is easier to complete the rolling of the beam in one heat because of the saving in time by the reduction in the number of passes thereby permitted.

The invention is not restricted to any particular number of passes for this widening and reducing operation, as this will necessarily be affected by the results aimed at in different cases and will depend on the condition of rolling and the products desired.

In the illustrative case, the passes succeeding the second pass in the first stand of rolls (see lower half of Fig. 1) are designed to work on the diagonally opposite flanges of the blank to thin them in sets of two in alternation, at the same time separating them somewhat and reducing the web to increase the depth and reduce the weight of the beam. For example, in the third pass the roll grooves 3, 3' are designed to work the top left and bottom right hand flanges and the return pass (4th) has roll grooves 4, 4' designed to work the unworked flanges in the third pass.

The diagonally opposite arrangement of working grooves enables the principal axial plane of the blank and grooves to be disposed at an inclination to the axis of rotation of the rolls, thereby permitting the blank to free itself more readily from the grooves, and thus relieves the guides and strippers. This arrangement is particularly advantageous in the rolling of double flanged shapes (such as I-beams) having thin flanges, for it tends to avoid stripping the flanges from the web at high rolling speeds.

The second stand of rolls (see Fig. 2) may be of any suitable type for reducing the blank to the desired shape for finishing. As illustrated, the roll passes are intended for a three-high mill, and the roll grooves 5, 5' and 6, 6' are shaped so as to work upon diagonally opposite flanges of the blank in an advantageous manner to thin and separate them, the reduction in area of the flanges and web in each pass being proportional. Part of the metal of the upper left and lower right flanges of the blank 17 (as seen in Fig. 2) is displaced sidewise by the grooves 5, 5' of the fifth pass and this increases the depth of the blank 18 therein formed; and a similar sidewise displacement of part of the metal of the opposite flanges is caused by the grooves 6, 6' of the return pass (6th) which still further increases the depth of the blank 19 formed therein.

Similarly, the roll grooves 7, 7', and 8, 8' of the seventh and eighth passes may advantageously be designed to work in succession upon the pairs of diagonally opposite flanges of the blank, at the same time sepa-

rating them somewhat and reducing the web in proportion to the reduction of the flanges, the grooves 7, 7' operating on one pair of flanges to produce the blank 20 and the 5 grooves 8, 8' operating upon the other pair of flanges to produce the blank 21 (see Fig. 4).

Rolling the flanges in alternation in this manner puts less strain upon the adjacent 10 ends of the web and hence contributes to the rolling of light sections having a thin web and thin flanges, and therefore is desirable, although not essential, to obtaining all the advantages of my invention.

15 The cross-sectional area and shape of the blank produced by the widening and reducing operations may be controlled to suit the desired finished beam so that the beam may be readily completed by a single finishing pass through a universal mill of well known construction, or by other well known rolling mill methods of finishing such beams. Although not essential to the successful practice of the invention, it is desirable from 20 the standpoint of cost that the various operations be performed at such speed that the billet may be broken down into a blank and rolled to the finished shape of the beam in one heat.

30 My invention is the first, so far as I am aware, that enables a thin web light weight beam to be completed at one heat, thus making it practical to produce such beams at a price that permits them to be sold in competition with wood joists and so-called metal lumber.

My invention has the further advantage, applicable to the production of all sizes and shapes of beams and girders, channels and 40 other rolled sections, of utilizing a narrower billet for wide and deep shapes than has heretofore been found practical, thereby not only reducing the rolling costs by lessening the reduction in area required, but also permitting the use of longer billets and thus expediting the heating and saving furnace space as well as facilitating handling in the earlier rolling operations.

It is obvious that the invention is not restricted to any particular shapes or dimensions of rolled beams and structural members, nor to the use of all of the steps described above in the illustrative process.

No claim is made herein to the light 55 weight beam produced by the practice of my invention, as that is the subject matter of another application for patent.

Having described an illustrative mode of practicing my invention, without limiting myself thereto, what I claim and desire to secure by Letters Patent is as follows:

1. The process of rolling which comprises a series of two or more similar operations involving lateral spreading of a suitable 65 billet or blank with comparatively slight re-

duction of cross-sectional area in proportion to the increase in width to produce a wide shallow section having short heavy flanges followed by repeated working of opposite sides to reduce and spread the flanges. 70

2. The process of rolling which comprises a series of two or more similar operations involving lateral spreading of a suitable billet or blank to produce a wide shallow section having short heavy flanges followed 75 by repeated working of opposite sides to reduce the web and flanges in proportion and spread the latter.

3. The process of rolling flanged members which comprises a series of two or more 80 similar operations involving lateral spreading of a suitable billet or blank to produce a wide shallow section with substantially flat sides followed by repeated working of opposite sides in progressively wider 85 grooves to reduce and spread the member from the middle toward the edges to separate the flanges thereby formed.

4. The process of rolling flanged members which comprises lateral spreading of a suitable billet or blank by wedging its margins away from its median vertical plane and flattening the connecting neck portion to produce a wide shallow section having short 90 heavy flanges followed by repeated working 95 of opposite sides to reduce the flanges and separate them.

5. The process of rolling flanged members which comprises lateral spreading of a suitable billet or blank by wedging its margins 100 away from its median vertical plane and flattening the connecting neck portion to produce a wide shallow section having short heavy flanges followed by repeated working 105 of opposite sides to reduce the flanges and separate them, said operations being performed with as little reduction in cross-sectional area as is consistent with filling the grooves of the rolls.

6. The process of rolling which comprises 110 repeated like operations operating principally upon the mid portion of a suitable billet or blank for laterally spreading it with comparatively slight reduction of 115 cross-sectional area in proportion to the increase in width to produce a wide shallow section having short heavy flanges.

7. The process of rolling flanged beams which comprises a series of rolling operations upon the mid portion of the blank to 120 groove it deeply and force the edges apart by wedge action followed by a series of rolling operations to reduce the web and flanges.

8. The process of rolling flanged beams 125 which comprises a series of like rolling operations upon the mid portion of the blank each operating to produce lateral spreading with comparatively slight reduction of area and large reduction of thickness as 130

compared with usual practise, whereby light weight beams having very thin webs may be produced.

9. The process of rolling flanged beams which comprises a series of like rolling operations upon the mid portion of the blank to produce lateral spreading with less than ordinary reduction of area and greater than ordinary reduction of thickness followed by a series of rolling operations to reduce the web and flanges thereby formed.

10. The process of rolling flanged beams which comprises a series of rolling operations principally upon the mid portion of the blank to groove it centrally and produce lateral spreading followed by a series of rolling operations upon alternate corners of the blank to reduce the web and flanges proportionally.

11. The process of rolling flanged beams which comprises a series of rolling operations principally upon the mid portion of the blank to groove it centrally and produce lateral spreading followed by a series of rolling operations upon alternate corners of the blank to spread the flanges and reduce the web and flanges proportionally.

12. The process of rolling flanged beams which comprises a series of rolling operations performed principally upon the mid portion of the blank to groove it centrally and produce lateral spreading with minimum reduction of area followed by a series of rolling operations upon alternate corners of the blank to reduce the web and flanges proportionally.

13. The process of rolling a flanged member of considerably greater depth than width from a billet of much less width than the depth of said member, which comprises passing said billet through a wide roll pass having working collars centrally of the grooves engaging the upper and lower faces of said billet along the mid-line and thereby channeling said billet and spreading the edges to form flanges, said spreading being carried to a width 30 to 50 per cent greater than that of said billet with a small reduction of cross-sectional area compared to the change in shape.

14. The process of rolling a flanged member of considerably greater depth than width from a billet of much less width than the depth of said member, which comprises passing said billet through a wide roll pass having grooves provided with circumferential

wedge shape working collars for engaging the upper and lower faces of said billet along the mid-line and thereby channeling said billet and spreading the edges apart to form flanges.

15. The process of rolling a flanged member of considerably greater depth than width from an approximately equal sided billet of much less width than the depth of said member, which comprises passing said billet through a wide roll pass having grooves with middle wedge portions engaging the upper and lower faces of said billet along the mid-line and thereby channeling said billet and spreading the edges apart to form flanges with a minimum reduction of cross-sectional area.

16. Rolling a light weight I-beam from a billet by passing the billet through grooved spreading rolls of considerably greater width than the billet, followed by elongating the flanged blank thereby formed by passing it through grooved reducing rolls having alternating working and comparatively non-working grooves to widen and thin the web and flanges, substantially as described.

17. Rolling a light weight I-beam of disproportionately great depth from a small billet or blank by first channeling and spreading it laterally in suitable spreading rolls so that it may then be rolled to final shape by reducing and elongating the web and flanges proportionally, substantially as described.

18. Rolling a flanged shape of the character described by first channeling centrally and thereby spreading a narrow billet to form a blank with relatively short flanges and then rolling the flanges and web of the blank to thin and extend them.

19. Rolling a flanged shape having a thin web in proportion to its depth from a bloom or billet having a height approximately the same as or less than its width and a width less than 70% of the depth of the finished shape by a spreading and reducing process of the character described.

20. Rolling a light weight flanged shape having a web thickness substantially less than heretofore from a bloom or billet in one heat by a spreading and reducing process of the character described.

In testimony whereof, I have signed my name to this specification.

NORMAN C. RENDLEMAN.